

May 23, 1972

H. GRAEFEN ET AL

3,664,831

LEAD ALLOYS HAVING IMPROVED CORROSION RESISTANCE

Filed March 17, 1970

2 Sheets-Sheet 1

FIG. 1



INVENTORS:

HUBERT GRAEFEN  
DIETER KURON

BY: *Johnston, Root, O'Keefe, Leif, Thompson & Schuttler*  
ATT'YS

May 23, 1972

H. GRAEFEN ET AL

3,664,831

LEAD ALLOYS HAVING IMPROVED CORROSION RESISTANCE

2 Sheets-Sheet 2

Filed March 17, 1970

FIG. 2



INVENTORS:

HUBERT GRAEFEN  
DIETER KURON

BY: *Johns, Toy, Root, O'Leiffe, Keif, Thompsons, Shurtliff*  
ATT'YS

1

3,664,831

## LEAD ALLOYS HAVING IMPROVED CORROSION RESISTANCE

Hubert Graefen, Lampertheim, and Dieter Kuron, Mannheim, Germany, assignors to Badische Anilin- & Soda-Fabrik Aktiengesellschaft, Ludwigshafen am Rhine, Germany

Filed Mar. 17, 1970, Ser. No. 20,179  
Claims priority, application Germany, Mar. 20, 1969,  
P 19 14 210.0  
Int. Cl. C22c 11/00

U.S. Cl. 75—166

5 Claims

### ABSTRACT OF THE DISCLOSURE

Lead alloys distinguished by improved corrosion resistance, particularly against sulfuric acid, and improved creep resistance. Suitable alloys of this kind are lead alloys containing—besides components for reducing grain size, assisting the formation of protective layers and increasing creep resistance, such as copper, nickel, tellurium and tin—at least 0.05% of palladium based on the total weight of the alloy.

This invention relates to lead alloys having improved corrosion resistance, particularly against sulfuric acid, and improved creep resistance.

Due to the generally good corrosion resistance of lead and lead alloys to sulfuric acid, liquids containing sulfuric acid and to sulfate-containing solutions, apparatus and other plant parts made of lead or lead alloys or provided with lead linings are used in industry on a large scale.

The range of possible applications of lead and lead alloys available at present is restricted, from the corrosion point of view, by the dissolution of the lead which increases with increasing concentration and increasing temperature of the sulfuric acid. One such limit for the use of lead has hitherto been set by 45% boiling sulfuric acid for example. The range of applications is also restricted, from the point of view of tenacity, by the relatively poor creep resistance of the previously known leads and lead alloys even at only moderately elevated temperatures.

The corrosion resistance of lead and lead alloys to sulfuric acid is due to the formation of a protective layer of lead sulfate. To enable such a protective layer to be formed, a corrosion process must first take place, which is then reduced to a small corrosion rate by the formation of the protective layer of lead sulfate. On account of the relatively high hydrogen overpotential of lead, however, the formation of a protective layer on pure lead is delayed or completely suppressed. For this reason it is known, for example, to add alloying components such as copper or nickel to the lead, as such components have a low hydrogen overpotential, that is, a higher effective current density. The corrosion of commercially pure lead (Pb 99.985%) and commercial lead alloys (Pb 99.9%, Cu; hard lead—1.5% Sb) by 50% and 70% boiling sulfuric acid solutions is given in Table 1 in mm./year.

TABLE 1.—CORROSION BEHAVIOR OF COMMERCIALLY PURE LEAD AND COMMERCIAL LEAD ALLOYS

| Alloy                    | Linear corrosion rate in mm./year in boiling sulfuric acid having a concentration of— | 50%  | 70% |
|--------------------------|---------------------------------------------------------------------------------------|------|-----|
| Pb 99.985.....           | 0.97                                                                                  | (1)  |     |
| Pb 99.9 Cu.....          | 0.48                                                                                  | 4.23 |     |
| Hard lead (1.5% Sb)..... | 0.41                                                                                  | 1.25 |     |

<sup>1</sup> Complete dissolution.

2

However, not only the magnitude of the hydrogen overpotential of the alloying component is responsible for rapid and effective formation of the protective sulfate layer, but also the size of the cathode area formed, which in turn depends on the solubility and distribution of the alloying component.

Research on the influence of cathodically effective alloying components has shown, surprisingly, that lead alloys have much greater corrosion resistance, particularly against sulfuric acid, and greatly increased creep resistance when they contain, in addition to alloying components for reducing grain size, assisting the formation of protective layers and increasing creep resistance, such as copper, nickel, tellurium and tin, at least 0.05%, preferably from 0.1 to 0.2%, of palladium based on the total weight of the alloy.

Such small additions of palladium to the commercial lead-copper alloy Pb 99.9 Cu greatly reduce their rates of corrosion in 50% and 70% sulfuric acid, as may be seen from Table 2, line 1. Moreover, we have found that the addition of at least 0.05% (preferably from 0.1 to 0.2%) of palladium to lead alloys already containing from 0.05 to 0.15% of nickel and from 0.1 to 0.15% of tin, lead alloys already containing from 0.05 to 0.15% of nickel and from 0.1 to 0.15% of tin and lead alloys already containing from 0.05 to 0.15% of tellurium and from 0.1 to 0.2% of tin causes a further surprising increase in the corrosion resistance (see Table 2, lines 2 to 5) and an unexpected improvement in their creep resistance compared with previously known lead alloys. For economic reasons, the concentration of palladium in the lead alloys will be kept as low as possible.

TABLE 2.—CORROSION BEHAVIOR OF LEAD ALLOYS ACCORDING TO THE INVENTION

[The figures in brackets indicate the percentage concentration of the alloying components]

| Alloy                                 | Linear corrosion rate in mm./year in boiling sulfuric acid having a concentration of— |      |
|---------------------------------------|---------------------------------------------------------------------------------------|------|
|                                       | 50%                                                                                   | 70%  |
| Pb, Cu, Pd (0.05, 0.1).....           | 0.02                                                                                  | 0.23 |
| Pb, Cu, Sn, Pd (0.05, 0.12, 0.1)..... | 0.10                                                                                  | 0.10 |
| Pb, Sn, Pd (0.10, 0.13, 0.2).....     | <0.01                                                                                 | 0.05 |
| Pb, Ni, Sn, Pd (0.08, 0.12, 0.1)..... | 0.015                                                                                 | 0.08 |
| Pb, Te, Sn, Pd (0.05, 0.11, 0.1)..... | 0.01                                                                                  | 0.07 |

FIG. 1 shows the creep curves of commercially pure lead (Pb 99.985), commercial lead-copper alloy (Pb 99.9 Cu), a lead-copper-palladium alloy according to the invention and a lead-copper-tin-palladium alloy according to the invention. The test temperature is 40° C., and the alloys were subjected to loads of 0.6 kg./mm.<sup>2</sup> and 0.4 kg./mm.<sup>2</sup>. The Brinell hardness of these alloys, as measured with a ball 2.5 mm. in diameter under a load of 3.1 kg. for a period of 120 seconds is 3.6, 3.6, 4.6 and 6.5 kg./mm.<sup>2</sup> respectively.

The samples of pure lead (Pb 99.985) broke under a load of 0.6 kg./mm.<sup>2</sup> after only about 2 hours and under a load of 0.4 kg./mm.<sup>2</sup> after about 75 hours (rupture indicated by x on the curves). The commercial lead-copper alloy (Pb 99.9 Cu) also broke under a load of 0.6 kg./mm.<sup>2</sup>. Samples of the lead-copper-palladium alloy (Pb 99.9 Cu+0.1 Pd) did not break when subjected to a load of 0.6 kg./mm.<sup>2</sup> for 700 hours, although the elongation had at this point exceeded 20%. The lead-copper-tin-palladium alloy, however, showed unexpectedly high creep resistance. After almost 1,000 hours under a load of 0.6 kg./mm.<sup>2</sup> this alloy showed an elongation of only about 2%. Under a load of 0.4 kg./mm.<sup>2</sup> the elongation was less than 1%.

In view of these results it appears advisable for the lead alloys of the invention to contain tin in addition to pal-

ladium. The addition of antimony, known from the literature as a method of increasing the tenacity of lead alloys, does not result in the same increase in creep resistance and corrosion resistance as the use of tin as alloying component.

FIG. 2 shows the quasi-stationary anodic current density/potential curves for the two commercial leads (Pb 99.985 and Pb 99.9 Cu) and the two lead alloys of the invention (Pb 99.9 Cu+0.1 Pd and Pb Cu Sn Pd (0.05; 0.12; 0.10)) in boiling 70% sulfuric acid. The current density/potential curves illustrate the two essential effects of the lead alloys of the invention responsible for the increase in corrosion resistance. On the one hand, the steady or corrosion potentials of the lead alloys of the invention have much higher positive values (+500 to +600 mv.), and on the other hand the constant dissolution current density is only about  $1 \times 10^{-5}$  amps./cm.<sup>2</sup> as against a value of about  $8 \times 10^{-4}$  for the commercial leads.

The addition of platinum or gold instead of palladium produces an improvement in corrosion resistance and creep resistance of the lead alloys but does not give the unusually good results obtained by adding palladium.

The main advantages of the lead alloys of the invention over the commercially available leads are their exceptionally high corrosion resistance especially to sulfuric acid and their exceptionally good creep resistance.

We claim:

1. Lead alloys having improved corrosion resistance, particularly against sulfuric acid, and improved creep resistance, which contain, in addition to such alloying

components as reduce grain size, assist the formation of protective layers and improve creep resistance, said alloying components selected from the group consisting of copper, nickel, tellurium and tin, a small amount of palladium, which is at least 0.5% based on the total weight of the alloy.

2. Lead alloys as claimed in claim 1 containing from 0.1 to 0.2% of palladium based on the total weight of the alloy.

10 3. Lead alloys as claimed in claim 1 containing from 0.05 to 0.15% of copper and from 0.1 to 0.15% of tin.

4. Lead alloys as claimed in claim 1 containing from 0.05 to 0.15% of nickel and from 0.1 to 0.15% of tin.

15 5. Lead alloys as claimed in claim 1 containing from 0.05 to 0.15% of tellurium and from 0.1 to 0.15% of tin.

#### References Cited

##### UNITED STATES PATENTS

|           |        |              |       |           |
|-----------|--------|--------------|-------|-----------|
| 2,145,513 | 1/1939 | Jones et al. | ----- | 75—166 EX |
| 2,171,180 | 8/1939 | Jones        | ----- | 75—166 EX |
| 2,348,333 | 5/1944 | D'Eustachio  | ----- | 75—166 D  |
| 3,147,114 | 9/1964 | Hack et al.  | ----- | 75—166 D  |

##### FOREIGN PATENTS

25 25 414,606 8/1934 Great Britain ----- 75—166 E

L. DEWAYNE RUTLEDGE, Primary Examiner

E. L. WEISE, Assistant Examiner

30 U.S. CL. X.R.  
75—166 D, 166 E

UNITED STATES PATENT OFFICE  
CERTIFICATE OF CORRECTION

Patent No. 3,664,831 Dated May 23, 1972

Inventor(s) Hubert Graefen and Dieter Kuron

It is certified that error appears in the above-identified patent  
and that said Letters Patent are hereby corrected as shown below:

Column 2, line 14, "elast" should read -- least --.

Column 4, line 5, claim 1, "0.5%" should read -- 0.05% --.

Signed and sealed this 20th day of November 1973.

(SEAL)

Attest:

EDWARD M.FLETCHER,JR.  
Attesting Officer

RENE D. TEGTMEYER  
Acting Commissioner of Patents